

# UNITED STATES PATENT OFFICE.

JONAS W. AYLSWORTH, OF EAST ORANGE, NEW JERSEY, ASSIGNOR OF ONE-HALF TO  
FRANK L. DYER, OF MONTCLAIR, NEW JERSEY.

## FIRE-EXTINGUISHING FLUID.

1,078,030.

Specification of Letters Patent.

Patented Nov. 11, 1913.

No Drawing.

Application filed January 23, 1913. Serial No. 743,843.

To all whom it may concern:

Be it known that I, JONAS W. AYLSWORTH, a citizen of the United States, and a resident of East Orange, in the county of Essex and 5 State of New Jersey, have invented certain new and useful Improvements in Fire-Extinguishing Fluids, of which the following is a description.

This invention relates to fluid compounds 10 for extinguishing fires of various natures, particularly those caused in whole or part by burning gasoline or other volatile liquids.

The object of the invention is to provide 15 an agent which shall more effectively extinguish such fires with a relatively small proportion of the extinguishing substance, which shall provide flame-extinguishing vapors at temperatures below the point at which gasoline and similar volatile liquids 20 begin to boil, and which preferably shall continue to evolve such vapors through a wide range of temperatures.

The compound is well adapted not only 25 for extinguishing fires in gasoline and the like, but also for smothering and putting out fires of various kinds, including electrical fires.

For extinguishing the flames of gasoline and the like, carbon-tetra-chlorid has previously been used with a fair degree of success. I have found, however, that a much 30 greater efficiency is secured in such cases if a liquid agent is used having a lower boiling point than the flaming liquid, or capable of 35 rapidly evolving flame extinguishing vapors at a temperature below the boiling point of the flaming liquid, and miscible with such liquid.

Carbon-tetra-chlorid is volatile and miscible 40 with gasoline, benzene and like substances, and is effective as a flame extinguisher therefor when a sufficient amount is used so that a sufficient quantity of vapor may be evolved to constitute a flame extinguishing atmosphere above and around the burning liquid. Carbon-tetra-chlorid however, and equivalent known extinguishing liquids, are much heavier and of higher boiling points than gasoline, for example, which 45 renders necessary the employment of a comparatively large amount of the extinguisher. I believe this to be because, first, the higher specific gravity of the substance, as carbon-tetra-chlorid, causes it when applied to a 50 gasolene fire for example, to first to a con-

siderable extent pass through the flaming fluid. An appreciable time then elapses before it becomes thoroughly mixed and appears at the surface and volatilizes. Secondly, the inflammable vapors of the gasoline are evolved more rapidly from the surface of the burning fluid than are the combustion-arresting vapors of the carbon-tetra-chlorid, and consequently a larger proportion of the extinguishing fluid must be used 60 than if the extinguisher volatilized readily at a lower temperature. Commercial gasoline, it should be remarked, is a mixture including various hydro-carbons of low boiling point, such as petroleum ether. On testing gasoline, I have found it to begin to boil at about 49° C. and between that temperature and 66° C., at which the gasoline was in considerable ebullition, a good deal of fluid had distilled over. Carbon-tetra-chlorid boils at about 76° C. 75

I overcome the above-described disadvantages by providing a liquid whose boiling point is lower than that of gasoline or other similar liquid. The substances which 80 I find effective as having the necessary low boiling point are, like carbon-tetra-chlorid, higher in specific gravity than gasoline although not so high as carbon-tetra-chlorid. Owing to their lower boiling points, however, they immediately get in violent ebullition upon striking the fire, and evolve vapors more rapidly than the gasoline, so that a much smaller proportion of these substances is required than of carbon-tetra-chlorid to produce the desired flame-extinguishing atmosphere. Liquids which I have 85 found to fulfil the above requirements are dichloro-ethane, (boiling point 36° C.), dichloro-methane (boiling point 41.8° C.), and di-chloro-ethylene (boiling point 55° C.), or admixtures of the same with carbon-tetra-chlorid or with each other. 90

In order that my composition may be applicable to fires of various natures, I prefer to compound the low-boiling-point liquid with carbon-tetra-chlorid, and also preferably with other bodies of higher boiling point than that of carbon-tetra-chlorid, for the purpose of furnishing flame-extinguishing vapors at higher temperatures after all the lower and more volatile liquids have been driven off. Such bodies, in solution or mixture with carbon-tetra-chlorid are described in my application Serial No. 498,358, 105 110

filed May 25, 1909, and are there described as perhalogenized organic radicals, such as perchlorinated naphthalene, di-phenyl, hexa-chloro-ethane, perchloro-tri-phenyl-benzene, hexa-chloro-benzene, etc. As stated in said application the carbon-tetra-chlorid volatilizes at a point which is sufficiently low, in the case of fires of various characters which are well under way, as to be expelled largely by the heat upon being applied to the fire, for which reason the higher boiling substances referred to were added. By compounding a substance such as di-chloro-ethane or methane, carbon-tetra-chlorid, and one or more of the higher-boiling point substances referred to above, I can obtain a liquid which evolves flame-extinguishing vapors over a range of temperature from below 60° C. to and over 315° C., all of which vapors form a smothering combustion-arresting dry blanket or atmosphere above and around the seat of combustion.

The ingredients described above may be used in various proportions through a considerable range. If carbon-tetra-chlorid and di-chloro-ethane or di-chloro-methane comprise the compound, substantially equal proportions give good results. The higher boiling point halogenized organic radical which may be dissolved in the carbon-tetra-chlorid may be for example, from 2 to 20 per cent. by weight of the carbon-tetra-chlorid.

When the compound is designed for general applicability it may also contain in suspension, certain metallic salts, such as finely divided tungstate of soda, which will deposit upon the charred carbon or substance burned, as a fire-proof coating, to retard the smoldering of the substance. Some of the perhalogenized organic constituent in solution, if the latter is used, such as perchlorinated naphthalene, is also thrown down on the burnt material as an electrically non-conducting deposit, which is of advantage in the case of electrical fires.

I determined by test that, to extinguish a given volume of burning gasolene, requires about an equal volume of carbon-tetra-chlorid. Less than one-fifth the volume of the gasolene of di-chloro-methane sufficed to extinguish the fire, under the same conditions, and about one-fifth the volume of the gasolene of a mixture of equal proportions of carbon-tetra-chlorid and di-chloro-methane sufficed.

In the term "perhalogenized organic radicals" mentioned above, I do not mean to limit myself to substances in which all the hydrogen has been replaced by chlorin or other halogen, but only to substances in which the greater part of the hydrogen has been so replaced.

The vapors of the substances described above are all non-poisonous, dry and combustion-arresting.

Having now described my invention what I claim as new and desire to protect by Letters Patent is:—

1. A flame extinguishing compound comprising a liquid the boiling point of which is lower than that at which gasolene begins to boil, together with a liquid the boiling point of which is higher than that of gasolene, both liquids being miscible with gasolene, and both, when sufficiently heated by being applied to a fire, evolving vapors to constitute a flame-extinguishing atmosphere above and around the seat of combustion. 70

2. A flame extinguishing compound comprising a chlorin derivative of a hydro-carbon having a boiling point lower than 60° C., compounded with a body having a boiling point higher than 60° C., said derivative and body, when applied to a fire, both evolving vapors to constitute a flame extinguishing atmosphere above and around the seat of combustion. 75

3. A flame-extinguishing compound comprising di-chloro-methane and carbon-tetra-chlorid. 80

4. A flame-extinguishing compound comprising a chlorin derivative of a hydro-carbon having a boiling point lower than that of gasolene, said derivative being miscible with gasolene, and carbon-tetra-chlorid. 85

5. A flame-extinguishing compound comprising di-chloro - methane, carbon - tetra-chlorid, and a perchlorinated organic radical having a boiling-point much higher than that of the carbon-tetra-chlorid. 90

6. A flame-extinguishing compound comprising di-chloro - methane, carbon - tetra-chlorid, and a halogenized benzene derivative dissolved in the carbon-tetra-chlorid and having a boiling-point much higher than that of the carbon-tetra-chlorid. 95

7. A flame-extinguishing compound comprising a liquid having the property when heated to a temperature below the boiling-point of gasolene, of rapidly evolving vapors to constitute a flame-extinguishing atmosphere, and of evolving further flame-extinguishing vapors when heated to temperatures above the boiling-point of gasolene. 100

8. A flame-extinguishing liquid compound comprising at least three ingredients, which boil at different temperatures, at least one of which is below 60° C., and at least one of which is much higher than that, and all of which, upon being volatilized, by application to a fire, evolve vapors to constitute a flame-extinguishing atmosphere above and around the seat of combustion. 105

9. A flame-extinguishing liquid comprising carbon-tetra-chlorid having dissolved therein a substance having a higher boiling point than that of the carbon-tetra-chlorid, compounded with a liquid having a lower boiling-point than carbon-tetra-chlorid, said substance and last named liq- 110

110

115

120

125

130

uid both having flame-extinguishing properties.

10. A flame-extinguishing liquid comprising an ingredient which boils and evolves flame extinguishing vapors at temperatures below 60° C., and ingredients which evolve flame extinguishing vapors only at higher temperatures, and a substance adapted to form a deposit upon the seat of combustion and retard the burning thereof.

11. A fire-extinguishing compound comprising a water-free liquid, miscible with

gasolene, having a boiling point lower than that of the lowest boiling point constituent of gasolene, and which is adapted, upon being applied to flaming gasolene, to evolve combustion-arresting vapors with greater rapidity than gasolene vapors are evolved.

This specification signed and witnessed this 21st day of January 1913.

JONAS W. AYLSWORTH.

Witnesses:

DYER SMITH,

SOPHIE M. BAEDER.